

W. F. FOX,  
 PHOTOGRAPHIC COLOR PRINT AND PROCESS OF PRODUCING SAME,  
 APPLICATION FILED MAR. 11, 1914.

1,166,121.

Patented Dec. 28, 1915.

NEGATIVE



Fig. 1

POSITIVE



Fig. 2,

Fig. 3,



PRINT FROM GREEN NEGATIVE

Fig. 4,



PRINT FROM RED POSITIVE

Fig. 5,



COLOR NEGATIVE

Fig. 6,



PRINT FROM RED POSITIVE

Fig. 7,



PRINT FROM GREEN POSITIVE

Fig. 8,



MONOCHROME NEGATIVE  
FROM RED AND GREEN POSITIVES

Fig. 10,



COLOR POSITIVE

Fig. 9,



MONOCHROME POSITIVE



Fig. 11,

WITNESSES  
*J. Mc. Inturh*  
*M. S. Gang*

INVENTOR  
*William Francis Fox*  
 BY  
*J. O. Edwards* ATTORNEY

# UNITED STATES PATENT OFFICE.

WILLIAM FRANCIS FOX, OF NEW YORK, N. Y., ASSIGNOR, BY DIRECT AND MESNE ASSIGNMENTS, OF TWO-THIRDS TO KINEMACOLOR COMPANY OF AMERICA, OF NEW YORK, N. Y., A CORPORATION OF DELAWARE.

## PHOTOGRAPHIC COLOR-PRINT AND PROCESS OF PRODUCING SAME.

1,166,121.

Specification of Letters Patent. Patented Dec. 28, 1915.

Application filed March 11, 1914. Serial No. 823,897.

To all whom it may concern:

Be it known that I, WILLIAM FRANCIS Fox, a subject of the King of Great Britain, and a resident of Beechhurst, in the 5 borough of Queens, city and State of New York, have invented certain new and useful Improvements in Photographic Color-Prints and Processes of Producing Same, of which the following is a specification.

10 The object of the invention is to produce photographs in substantially the natural colors of the original objects or scenes. Such invention is adapted for the production either of single color-photographs or of 15 extended series thereof capable of use, for example, in a suitable projecting-machine.

My invention relates chiefly to improved processes for producing photographic color prints.

20 It also comprises a photographic color print as an article produced by one form of my improved process.

In carrying out the invention, I make a photographic negative, in monochrome, 25 containing two images of a scene or object.

These images are taken through suitable color-filters, one being preferably green and the other red. As a result of the use of these filters, one of said images will faithfully 30 represent the subject-matter photographed, save that all red color-sensations will have been eliminated. In the other image, the subject-matter has also been faithfully portrayed, save that green color- 35 sensations have been eliminated. From the negative so obtained, I make a positive print, and such negative and positive are then used in the production of two additional negatives, which are subsequently

40 used for reproducing one of the two images in positive form in such manner that the image printed from one of said additional negatives may be supplied with color, while the image printed from the other negative 45 may be used to correct the positive image last referred to with respect to color gradations.

The invention is illustrated in the accompanying drawing, which is mainly diagrammatic.

50 In said drawing, Figure 1 is a plan view illustrating a negative film, and Fig. 2 a similar view of the positive film made therefrom, these portraying two crosses, one (the

left) in the original scene being of red 55 color, and the other of green, against a white background, the upper image of the negative film having been taken through a green color-filter, and the lower image through a red color-filter. Figs. 3, 4 and 60 5 are plan views, illustrating the production of what I term a "color-negative," i. e., a negative made from the "green image" of the negative shown in Fig. 1 and the "red image" of the positive shown in Fig. 2. 65 Figs. 6, 7 and 8 are plan views, illustrating the production of what I term a "monochrome negative," i. e., a negative in black-and-white made, by superimposed printing, from the red image upon the positive (Fig. 70 2) and from the green image upon the positive (Fig. 2). Fig. 9 is an edge view of a section of film provided with a coating of emulsion on each side thereof. Fig. 10 is a plan view of a positive image printed 75 from the color-negative (Fig. 5), and Fig. 11 is a similar view of a positive image printed from the monochrome negative (Fig. 8).

80 In the practice of the process under disclosure, I proceed first, as above indicated, to produce a negative film of not less than two images, using for this purpose preferably, although not necessarily, a consecutive-view camera provided with green and 85 red color-filters which are successively brought before the aperture. As a result, what I shall term herein the "green image" is an image of the subject matter, from which, however, red color-sensations have 90 been eliminated, while what I shall term herein the "red image" is an image of the subject matter, from which, however, green color-sensations have been eliminated. To aid in the disclosure, I have assumed in the 95 drawing that the subject-matter photographed comprised a white background and two crosses side by side, one of these (the left) being of red color and the other of green. The negative film A (Fig. 1), after 100 being developed and fixed in the usual manner, is used for the production, by the usual printing practice if desired, of a positive film B (Fig. 2). The negative and positive films so produced and which may, as 105 above indicated, contain either two or a greater number of images, are utilized for the production of what I term a "color-

negative" and a "monochrome negative," and by means of these is produced the positive constituting the finished product under this invention.

In producing the color-negative, I proceed as follows: In the first place, it will be understood, as above indicated, that in the finished product hereinafter described, the colors, on the image produced by the use of the color negative, representing the natural colors of the object photographed, are to be supplied by subjecting such image to the action of green and red coloring solutions, one of these being preferably a chemical reagent and the other a dye. It is desirable that in the image subjected to this treatment those portions adapted to take up the green color shall be represented by the silver deposit, and that those portions designed to take up the red color shall be represented by substantially clear gelatin. White and intermediate colors will be represented by both silver deposit and gelatin, but in varying quantity of the former, as a result whereof the portions so colored will take up to a sufficient extent for the purpose named either the green or the red.

Using the green image G of the negative A, I first obtain a print therefrom, indicated at C (Fig. 3). Here the green cross (at the right, Fig. 1) appears white, the red cross (at the left, Fig. 1) appears dark, and the background is substantially clear. Immediately over this image C, I print (see Fig. 4) the image of the red positive (R, Fig. 2), the lines of the images being, of course, in perfect registry. As a result, the red cross appears more intensely dark, the green cross remains white, and the background is gray. This is accomplished by regulating the time of exposure. As a result of the printing of the superimposed green negative image and red positive image (Figs. 3 and 4), I produce the "color-negative" D, (Fig. 5) in which the color gradations are directly opposite those which it is designed to produce on the finished product. In such color-negative, the background is gray, the green cross is white, and the red cross is intensely dark.

Having produced the color-negative, I now produce another negative, termed herein the "monochrome negative", since in the practice of the invention herein disclosed it is proposed that the ultimate positive print shall be, in practical effect, a composite consisting of a reproduction from the color-negative, modified or graded, however, by a reproduction from a negative in black-and-white. I proceed as follows:— Using the red positive (R, Fig. 2), I obtain a print E (Fig. 6) upon a film or other suitable substance. Here the background is gray, the green cross is clear, while the red cross also is gray. Next, using the green

positive image, (G, Fig. 2) I print the same (F, Fig. 7) directly over the print E (Fig. 6) made from the red positive image. In printing from the red positive R and the green positive G, I give each about one-half the normal or usual exposure. In effect, therefore, the two exposures equal one normal or usual exposure. The resultant image H (Fig. 8), constituting what I call the "monochrome negative", has these characteristics:—The background having been doubly printed is sufficiently dark to prevent an exposure being made through it in the subsequent printing step about to be described, while the two crosses are somewhat lighter, in order to permit these to be imprinted, during the next step of the process, upon the final film.

As previously explained, the image printed by the color-negative upon the final positive is subjected to color treatment, but the necessary color gradations not being present, correction, as by means of a monochrome negative, is desirable. To this end, I may use for the final product a film provided with emulsion on one side and the print from the color-negative may be impressed upon this, and then, after such print has been colored, the surface of the film may be waterproofed and over such waterproofed surface the film may be re-emulsified and a print from the monochrome negative impressed thereon in precise registry with the color-image. I prefer, however, to follow a somewhat different procedure, involving the use of a film having a coating of emulsion on both sides thereof, as illustrated at I, Fig. 9.

By suitable means, as by direct printing, and using the color-negative D, I obtain a print therefrom on one of the emulsified surfaces of the film I, the exposure being so regulated that the emulsion on the other side of said film will not be affected. By similar, or other desirable, means, and using the monochrome negative H, I obtain a print therefrom (regulating the exposure as above explained) on the emulsified surface of the film I opposite the surface upon which a print has been impressed by means of the color-negative D, being careful to observe that the prints formed by the use of both negatives are in perfect registry. The print obtained from the color-negative is illustrated in Fig. 10, while the print obtained from the monochrome negative is illustrated in Fig. 11.

The film bearing an image on either side thereof is now ready for development, and this may be accomplished by immersion in a suitable bath, development proceeding on both sides thereof simultaneously. After development, and the usual fixing, washing and drying, that side of the film bearing the print from the monochrome negative is

waterproofed in suitable manner, as, for instance, by the use of a suitable varnish or transparent celluloid.

The foregoing steps having been performed, the film is now ready for coloring by immersion in a suitable bath, the print from the monochrome negative being, as above indicated, protected during that operation. I first immerse the film in an acid green bath. A suitable bath may be compounded of the following constituents:—

|                                                |                |
|------------------------------------------------|----------------|
| Vanadium chlorid                               | 20 grains      |
| Ferric ammonium oxalate                        | 10 "           |
| Ferric chlorid                                 | 10 "           |
| 15 Potassium ferricyanid                       | 20             |
| Glacial acetic acid                            | 10 minimis     |
| Oxalic acid                                    | 100 grains     |
| Water sufficient to make the total composition | twenty ounces. |

20 Immersion of the film in this bath for five minutes will ordinarily be sufficient. After it has been removed from such bath, it may be washed to remove superfluous materials, after which to clear the image and make it more transparent it is immersed in an ordinary acid fixing bath, such as is commonly employed, and in this it is allowed to remain for a sufficient time to accomplish the purpose stated. Upon removal therefrom, the film may be washed sufficiently to remove sodium thiosulfate. The film is then immersed in a bath containing a suitable red dye, for instance an 25 anilin dye, and in this bath it is allowed to remain until any white object in the image shows white. The remaining colors will then be of correct intensity. After removal from the bath, the film may be rinsed to remove superfluous red dye, after which it is 30 dried and the process is then complete.

Throughout the foregoing specification, I have referred to the emulsion-bearing surface as a film, but it will, of course, be apparent that glass plates may be employed, particularly where the finished picture is to be used as a transparency. It will also be apparent that while the process is adapted for utilization to produce a single discrete print, it is also admirably adapted for use in consecutive-view color photography. In this, the common practice of employing color-filters during the projection of the pictures upon a screen is dispensed with, 35 since the colors are carried by the film itself. Also, the number of images necessary to produce an exhibition in color of given length is reduced by one-half, as compared with processes now in use since but one finished projecting positive picture will result from two images upon the original negative.

Having now described my invention, what I claim as new therein and desire to secure by Letters Patent is as follows:

65 1. A photographic process involving the

production of a negative of two images from one of which certain color sensations have been omitted and from the other of which certain other color sensations have been omitted, obtaining a positive print 70 from said negative on transparent or translucent material, producing by means of said negative and positive a second negative, obtaining a positive print from said second negative, obtaining from said first named 75 positive print a third negative and impressing upon sensitized material a print from each of said second and third negatives in registry with each other, substantially as set forth.

2. A photographic process involving the production of a negative of two images from one of which certain color sensations have been omitted and from the other of which certain other color sensations have 80 been omitted, obtaining a positive print from said negative on transparent or translucent material, producing a second negative by the use of that image of the original negative from which certain color sensations 85 have been omitted and that image of said positive print from which other color sensations have been omitted, obtaining a positive print from said second negative, obtaining from said first named positive print a third 90 negative and impressing upon sensitized material a print from each of said second and third negatives in registry with each other, substantially as set forth.

3. A photographic process involving the production of a negative of two images from one of which certain color sensations have been omitted and from the other of which certain other color sensations have been omitted, obtaining a positive print from said negative on transparent or translucent material, producing by means of said negative and positive a second negative, obtaining from said first named positive print a third negative, printing from said second negative upon sensitized material, printing on said material in registry with the print so obtained the image of said third negative and coloring one of the prints from said last named negatives, substantially as set forth.

4. A photographic process involving the production of a negative of two images from one of which certain color sensations have been omitted and from the other of which certain other color sensations have 115 been omitted, obtaining a positive print from said negative on transparent or translucent material, producing by means of said negative and positive a second negative, obtaining from said first named positive print a third negative, printing from said second negative upon one side of a surface which has been sensitized on both sides, superimposing on the print so obtained, but on the opposite side of said surface, the image of 120

125

130

said third negative and coloring one of the prints made from said last named negatives, substantially as set forth.

5. A photographic process involving the production of a negative of two images from one of which certain color sensations have been omitted and from the other of which certain other color sensations have been omitted, obtaining a positive print 10 from said negative on transparent or translucent material, producing by means of said negative and positive a second negative, obtaining from said first named positive print a third negative, printing from 15 said second negative upon one side of a surface which has been sensitized on both sides, superimposing on the print so obtained, but on the opposite side of said surface, the image of said third negative, developing 20 both prints, protecting one of them, by waterproofing, and coloring the other, substantially as set forth.

6. A photographic process involving the production of a negative of two images 25 from one of which certain color sensations have been omitted and from the other of which certain other color sensations have been omitted, obtaining a positive print from said negative on transparent or translucent material, producing by means of said negative and positive a second negative, obtaining from said first named positive print a third negative, printing from 30 said second negative upon one side of a surface which has been sensitized on both sides, superimposing on the print so obtained, but on the opposite side of said surface, the image of said third negative, developing both prints, 35 protecting one of them by waterproofing, and coloring the unprotected print by immersing it in color baths, substantially as set forth.

7. A photographic process involving the production of a negative of two images 45 from one of which certain color sensations have been omitted and from the other of which certain other color sensations have been omitted, obtaining a positive print from said negative on transparent or translucent, material, producing by means of said negative and positive a second negative, obtaining from said first named positive print a third negative, printing from 50 said second negative upon one side of a surface which has been sensitized on both sides, as by gelatin-silver emulsion, superimposing on the print so obtained, but on the opposite side of said surface, the image of said third negative, developing both 55 prints, protecting one of them, by waterproofing, and subjecting the other to solutions one of which will color those portions of the print represented by silver deposit

and the other of which will color those portions of the film which are clear, substantially as set forth. 65

8. A photographic process involving the production of a negative of two images from one of which certain color sensations have been omitted and from the other of which certain other color sensations have been omitted, obtaining a positive print 70 from said negative on transparent or translucent material, producing by means of said negative and positive a second negative, obtaining from said first named positive print a third negative, printing from 75 said second negative upon one side of a surface which has been sensitized on both sides, superimposing on the print so obtained, but on the opposite side of said surface, the image of 80 said third negative, developing both prints, protecting one of them by waterproofing, and subjecting the other to treatment in a toning bath and a dyeing bath, substantially as set forth. 85

9. A photographic process involving the production of a negative of two images from one of which certain color sensations have been omitted and from the other of which certain other color sensations have been omitted, obtaining a positive print from said negative on transparent or translucent material, producing by means of said negative and positive a second negative, obtaining from said first named positive print a third negative, printing from 90 said second negative upon one side of a surface which has been sensitized on both sides, superimposing on the print so obtained, but on the opposite side of said surface, the image of 95 said third negative, developing both prints, protecting one of them by waterproofing, and subjecting the other to treatment in a toning bath and a dyeing bath, substantially as set forth. 100

10. A photographic print of transparent 110 or translucent material, coated on both sides, each side bearing a photographic image, one being a monochrome print, and the other a color print, having colors corresponding to the color elements of the object photographed, said prints representing the same object and being in registration with each other, and said monochrome print having a waterproof transparent coating over the same, substantially as set forth.

This specification signed and witnessed this 9th day of March, 1914.

WILLIAM FRANCIS FOX.

Witnesses:

S. O. EDMONDS,  
I. MCINTOSH.